

May 7, 1963

J. P. KNUDSEN  
MANUFACTURE OF SHAPED OBJECTS OF ACRYLONITRILE  
POLYMER BY WET SPINNING

3,088,188

Filed Jan. 4, 1960

3 Sheets-Sheet 1



INVENTOR.  
JOHN PETER KNUDSEN

BY *Stanley M. Tarter*

ATTORNEY

May 7, 1963

J. P. KNUDSEN  
MANUFACTURE OF SHAPED OBJECTS OF ACRYLONITRILE  
POLYMER BY WET SPINNING

3,088,188

Filed Jan. 4, 1960

3 Sheets-Sheet 2



FIG. 5.



FIG. 6.



FIG. 7.



FIG. 8.

INVENTOR.  
JOHN PETER KNUDSEN  
BY  
*Stanley M. Taylor*  
ATTORNEY

May 7, 1963

J. P. KNUDSEN  
MANUFACTURE OF SHAPED OBJECTS OF ACRYLONITRILE  
POLYMER BY WET SPINNING

3,088,188

Filed Jan. 4, 1960

3 Sheets-Sheet 3



FIG. 9.



FIG. 10.



FIG. 11.

INVENTOR.  
JOHN PETER KNUDSEN

BY *Stanley M. Tarter*

ATTORNEY

## 1

3,088,188

**MANUFACTURE OF SHAPED OBJECTS OF ACRYLONITRILE POLYMER BY WET SPINNING**  
John P. Knudsen, Decatur, Ala., assignor, by mesne assignments, to Monsanto Chemical Company, a corporation of DelawareFiled Jan. 4, 1960, Ser. No. 314  
14 Claims. (Cl. 28—32)

This invention relates to improved shaped objects such as fibers, filaments, yarns and the like manufactured from acrylonitrile polymers and to an improved process of producing same. More particularly, this invention concerns such shaped objects having a normally lustrous appearance and possessing an optimum balance of longitudinal and lateral properties and a process for producing same.

In view of the thermal instability of acrylonitrile polymers, filaments of such polymers are formed by dissolving the polymers in a suitable solvent and then removing the solvent from a flowing stream of the solution to form filaments therefrom. Commercially, filaments of acrylonitrile polymers are prepared either by the dry spinning process or by the wet spinning process, as is well known. The specific technique chosen results in a compromise among the yarn properties, the economic aspects of the techniques involved, and other considerations. There are advantages and disadvantages associated with the employment of each process.

The present invention is particularly concerned with the wet spinning process. Ordinarily, in a wet spinning operation coagulation is accomplished by extruding the polymer solution into an aqueous bath sometimes containing a percentage of solvent or dissolved salt. As used herein an aqueous or water bath refers to a composition having water as one of its main components. When the solvent is extracted from the extruded stream of spinning solution in a coagulating bath during wet spinning, solidification of the polymer in filamentary form results. Normally, during coagulation there is an inward diffusion of coagulating bath liquid into the filaments undergoing coagulation, as well as a corresponding outward movement of solvent into the coagulating bath. The solvent and the bath liquid may interchange in such a manner that the resulting filaments contain voids or cavities along their lengths which can be seen clearly with an optical phase microscope. Filaments containing these voids or unfilled spaces do not possess the requisite physical properties desired for some end uses. For example, such filaments exhibit a delustered appearance, lower tenacity, and lower abrasion resistance as compared with filaments not containing voids.

To overcome this physical weakness inherently formed in the filaments, positive aftertreatment steps during the processing of the filaments normally are taken. The tenacity of the filaments is improved greatly by various modes of stretching that molecularly orient the polymer molecules but which in addition tend to collapse these voids. To collapse fully these voids the filaments may be dried at rather high temperatures under tension, thereby forming a more dense filamentary structure. The prior art has found that the tenacity of the filaments is satisfactory with such aftertreatment of the filaments. However, tenacity is primarily a longitudinal property of the filaments; and satisfactory tenacity is not the full answer to the attainment of filaments having an optimum balance

## 2

of properties. In many end uses the abrasion resistance and the resistance to break upon being flexed (flex life) are most important. Such properties may be regarded as lateral properties as distinguished from longitudinal properties. While drying under tension gives the illusion of forming filaments without voids therein, the voids merely are crushed together. Although the crushed voids do not detract from the longitudinal properties of the filaments to any significant extent, it has been found that lateral stresses cause the filaments to splinter or break. In other words, filaments having voids which are merely crushed together are laterally weak. The art has found that the lateral properties of the filaments can be improved substantially by subjecting the filaments to an annealing operation. One such annealing procedure includes a series of elevated and reduced pressure treatments applied to the filaments. More specifically, annealing can be accomplished by placing the acrylonitrile polymer filaments in a closed chamber, subjecting them to a high temperature and pressure in the presence of wet steam and then evacuating the chamber. This treating cycle is repeated as many times as needed. It will be appreciated that this annealing operation as just described is expensive and time consuming. Omitting the annealing step in the aftertreatment of the wet spun acrylic filaments results in filaments having a tendency to splinter or fibrillate; and hence, the filaments have a low abrasion resistance. This tendency to fibrillate is minimized by annealing the filaments. The improvement is thought to result from the interface surfaces of the collapsed voids being rendered less separable.

In addition to the possible presence of the voids which are visible under an optical phase microscope and occur in filaments of acrylonitrile polymers coagulated in an aqueous coagulating bath, electron microscopy has shown the existence of a reticulate structure in the filaments displaying a network of submicroscopic pores or interstitial spaces most of which intercommunicate with each other. These pores in freshly spun filaments, that is filaments which have been coagulated without having been subjected to any aftertreatment producing a pronounced change in the structure thereof, are quite observable under an electron microscope. The polymers comprising the filaments appear to take the form of a latticework of integrally joined strings. The polymer lattice has a pattern resembling that of a fine, extremely small meshwork, although the interstices are usually somewhat irregular in size and shape. The microspores present in filaments produced by ordinary wet spinning techniques as they leave the coagulating bath are more or less spherical with the polymer lattice defining such interstitial spaces. The distances across these spaces are ordinarily about 250 Å. to 3000 Å. or greater. The frequency of occurrence of the micropores in the filaments produced by ordinary wet spinning techniques employing aqueous coagulating baths can be estimated under an electron microscope and is usually  $35-90 \times 10^{14}$  per gram of polymer. The presence of these pores is believed to explain the anomalously low density of normal filaments as they leave the coagulating bath. At this point the apparent density of the filaments produced by ordinary wet spinning techniques employing aqueous coagulating baths is usually about 0.4 to 0.5 gram per cubic centimeter.

It will be appreciated that the voids that are visible under the optical phase microscope are quite different from the micropores or interstitial spaces not visible under an optical phase microscope but readily apparent under an electron microscope. Hence, the term "voids" as used

herein signifies enclosed spaces or surface pits of the filaments which are visible under an optical phase microscope and which do not contain acrylonitrile polymer, whether or not the enclosed spaces contain a fluid or are collapsed. The term "micropore" as used herein signifies extremely diminutive enclosed spaces or surface pits of the filaments that are not visible under an optical phase microscope but are visible under an electron microscope and that do not contain acrylonitrile polymer, whether or not the enclosed spaces contain a fluid or are collapsed.

When the freshly spun filaments are stretched, these micropores as would be expected assume the geometric configuration of an ellipsoid. Subsequent collapsing of the porous structure of the filaments due to the presence of these micropores can be accomplished by drying the filaments under tension at an elevated temperature. Annealing the filaments renders the interstitial interface surfaces of the micropores less separable. Hence, annealing is regarded as an important step in the attainment of acceptable lateral physical properties in the filaments.

In accordance with one aspect of the present invention the size and frequency of the interstitial spaces are correlated with each other so as to produce filaments offering an optimum combination of longitudinal and lateral properties. Therefore, a method is provided whereby the size and frequency of the normally occurring micropores are changed substantially to produce filaments having such properties.

It is an object of this invention to provide filaments and the like of acrylonitrile polymers that possess an advantageous combination of lateral and longitudinal physical properties.

Another object is to provide a process for producing such filaments by modification of the conventional acrylonitrile polymer filament forming processes.

Other objects will become apparent from the following description of the invention and claims.

In general, these objects are accomplished in accordance with the invention by continuously extruding a solution of an acrylonitrile polymer through a desired number of orifices in a spinneret disposed in a liquid medium composed of polyalkylene glycol and continuously directing the thus-formed streams of the solution for a short distance through the medium to coagulate the polymer in the form of filaments. The solvent employed is N,N-dimethylacetamide, N,N-dimethylformamide or the like. The coagulating bath preferably is composed essentially of polyalkylene glycol although during spinning the solvent concentration will build up in the bath with certain concentrations of solvent being completely tolerable. Fresh coagulating bath composition should be supplied to the coagulating bath when the solvent concentration therein becomes excessively high. The solvent is recovered from the bath by conventional methods. Up to at least 20% concentration by weight of solvent can ordinarily be tolerated in the coagulating bath without adversely affecting the filament appearance or properties. Although the coagulating bath is preferably free of water, nevertheless, water may be present in the coagulating bath in minor amounts without inducing the formation of inferior filaments. For best results, it is necessary to maintain the water concentration in the coagulating bath below 10%. When greater amounts of water are present in the coagulating bath, inferior filaments may be produced. By employing the spinning composition composed of acrylonitrile polymer dissolved in N,N-dimethylformamide, N,N-dimethylacetamide or the like and spinning such composition into a polyalkylene glycol coagulating bath, the filaments produced possess advantageous physical properties and differ in structure from other acrylonitrile polymer filaments heretofore known in the art. During their travel from the spinneret to the means used to withdraw the filaments from the coagulating bath, a stretch may be imparted to the filaments in order to attenuate same, if desired. After being removed from the

coagulating bath the filaments are stretched to obtain a desired orientation according to various techniques in order to increase the tenacity, as well as otherwise to improve the physical properties of the filamentary material. 5 Although the orientation stretch may be accomplished in various ways, it is preferred that the filaments after being withdrawn from the coagulating bath be continuously directed through a second bath and stretched therein. This second bath is preferably composed of hot water; additional solvent remaining in the coagulated filaments is removed therefrom in the second bath. Following this operation the filaments optionally may be continuously permitted to relax under low tension or in a hot liquid or hot gaseous atmosphere and/or then continuously dried. 10 In addition to the stretching operation other treating and processing steps may be given the filaments, such as for example, washing, crimping, cutting into staple lengths. The filaments may be collected in continuous form or in staple form. Of course, various lubricants and other beneficial treating agents may be advantageously placed on the fibers during the manufacturing operation.

To further understand the invention reference will be made to the attached drawing that forms part of the present application.

In the drawing,

FIGURE 1 is a side elevational view partly in section showing schematically an apparatus arrangement of a type which can be used in carrying out the process of the present invention;

FIGURE 2 is a reproduction of a photomicrograph at a magnification of about 100 times of acrylonitrile polymer filaments of textile grade which give the appearance of smooth, glassy rods;

FIGURE 3 is a reproduction of a photomicrograph of greater magnification of an acrylonitrile polymer filament that contains numerous voids along the length thereof;

FIGURE 4 is a reproduction of a photomicrograph of an acrylonitrile polymer filament substantially free of voids;

FIGURE 5 is an electron micrograph of 41,000 times magnification illustrating in longitudinal section the microporous structure existing in the novel freshly-spun filaments herein;

FIGURE 6 is an electron micrograph of 44,000 times magnification illustrating in longitudinal section the microporous structure existing in the freshly-spun filament in FIGURE 5 after same has been given an orientation stretch of 6 times;

FIGURE 7 is an electron micrograph of 41,000 times magnification illustrating in longitudinal section the microporous structure existing in heretofore known freshly-spun filaments;

FIGURE 8 is an electron micrograph of 44,000 times magnification illustrating in longitudinal section the microporous structure of the filament shown in the just preceding figure after same has been given an orientation stretch of 6 times;

FIGURE 9 is an electron micrograph of 26,000 times magnification illustrating in longitudinal section the structure and surface of wet-spun oriented filaments heretofore known and collapsed by being dried under tension;

FIGURE 10 is an electron micrograph of 26,000 times magnification illustrating the frayed surface structure of the filament in FIGURE 9 after same has been subjected to lateral stresses; and

FIGURE 11 is an electron micrograph of 11,000 times magnification illustrating the contrasting difference between voids and micropores existing in freshly-spun acrylonitrile filaments.

The present invention provides novel filaments which differ markedly from previous wet-spun acrylonitrile polymer filaments.

The novel filaments of the present invention are of textile grade quality and are molecularly oriented. The

term "textile grade quality" refers to the characteristics required of textile filaments, fibers, and the like with respect to strength, elongation, etc. in order that the same can be converted into an acceptable fabric. The filaments also are manufactured from an acrylonitrile polymer and are substantially free of porosity. To be substantially free of porosity means that the density of the filaments closely approaches or corresponds with the density of the acrylonitrile polymer from which the filaments are produced. The filaments are particularly characterized by displaying an internal fiber surface area in the range of about 150-500 square meters per gram of filament. The inner surface area of the filaments is the total surface area thereof less the geometric external surface area thereof and is measured as described more fully below. The inner surface area is therefore an indication of the number of the micropores in the reticulate filamentary structure. This area is best seen and measured by analyzing a sample of the coagulated filaments as they leave the coagulating bath. In view of the fact that the micropores in the final filamentary structure appear to be matted together, the inner surface area is actually a measure of the total area of the engaging surfaces defining collapsed submicroscopic interstitial spaces. In addition the filaments are characterized by having the interstitial spaces spaced apart at a distance of from 10 Å. to at most about 300 Å. as measured before the filaments are oriented and before said spaces are collapsed. That is to say, that assuming the micropores take the form of a sphere, the average diameter of the micropores before orientation and collapsing is 300 Å. or less as can be measured visually under an electron microscope. Furthermore, the frequency of the interstitial spaces in the filaments is in the range of about  $200-2000 \times 10^{14}$  per gram of filament which can be calculated from internal surface area and diameter data or estimated by visual analysis. The average number of interstitial spaces in the filaments is at least 40,000 per millimeter of length. The filaments may be further characterized by having at least as good and in most instances a higher resistance to abrasion when wet than dry. The novel filaments require a relatively high tension in order to be elongated. For example, a tension of at least one gram per denier has been found to be necessary to elongate a given filament 5 percent in water at 100° F. Comparably high tensions are required at other temperatures to elongate the filaments. The apparent density of the filaments leaving the coagulating bath is unusually high in that they exhibit densities of about 0.7 to almost 1.0 gram per cubic centimeter. Also at this point the filaments have an area ratio of 1.5 to 1.1. Hence, by having such a high density, ab initio, i.e. early in the production of the filaments, some of the conventional aftertreating steps that induce the formation of a denser structure, such as relaxing and annealing described-above can be omitted, if desired, without substantial loss of properties.

It is known that all solids have adsorbed gases on their surfaces at all temperatures and pressures. As the temperature is lowered and the pressure is increased, the amount of gas adsorbed thereon increases. The amount of gas adsorbed can be quantitatively measured if it is large enough. Hence, methods of low temperature gas adsorption for the determination of the surface area of porous solid samples are known. The usual studies of gas adsorption are isothermal rather than isobaric because of the relative ease of maintaining constant temperature and variable pressure conditions.

The experimental determination of the isothermal volume of gas adsorbed as a function of pressure gives rise to one of five classical types of isotherms. The shapes of the isotherms are a function of the size of the adsorbing molecule. In the gaseous adsorption method the gas condenses on the surfaces of the sample whose surface area is being measured and gradually covers the surface as the pressure is increased until a monolayer of gas is

adsorbed thereon. Further increases in pressure result in progressive increases in the thickness of the adsorbed layer until at a partial pressure of one, the adsorbed phase is indistinguishable from the liquid phase of the gas.

5 Provided that the volume of gas adsorbed at the monolayer point and the cross sectional area of the gas molecule are known, the surface area can be calculated. The advantage of using gas molecules is that the individual gas molecules are small enough to fill the micropores of the novel filaments herein, the diameter of which is only a few angstroms larger than that of the gas molecule.

10 15 The Brunauer-Emmett-Teller (BET) theory of multilayer physical adsorption described in numerous printed papers is regarded to be the most generally applicable theory explaining the isothermal adsorption of a gas on a free surface of a solid. The following expression for such isothermal adsorption is obtained by application of the BET theory:

$$20 V = \frac{V_m CP}{[P_0 - P] \left[ 1 + (C-1) \frac{P}{P_0} \right]} \quad (1)$$

25 wherein  $V$  is the volume of gas adsorbed at a particular pressure  $P$ ,  $C$  is a constant related to the heat of adsorption,  $V_m$  is the volume of gas adsorbed for a monolayer,  $P_0$  is the saturation pressure of the gas at the temperature of the experiment, and  $P/P_0$  is defined as the relative pressure.

30 35 Of the terms appearing in (1)  $V$ ,  $P$ , and  $P_0$  are experimental;  $V_m$  and  $C$  are characteristic of the system under study. By rearrangement, Equation 1 can be put in the form:

$$\frac{P}{V(P-P_0)} = \frac{1}{V_m C} + \frac{C-1}{V_m C} \frac{P}{P_0} \quad (2)$$

so that a plot of

$$\frac{P}{V(P-P_0)} \text{ vs. } \frac{P}{P_0}$$

40 45 should give a straight line with a slope ( $S$ ) of

$$\frac{C-1}{V_m C}$$

and an intercept ( $I$ ) of

$$\frac{1}{V_m C}$$

These two equations can be solved to give

$$50 V_m = \frac{1}{S+1} \quad \text{and} \quad C = \frac{S}{I} + 1$$

For most isotherms a linear plot is obtained only for the region of 0.05 to 0.40 relative pressure units. This range is more than sufficient for a satisfactory determination of  $V_m$ .

55 60 The cross sectional area of the gas molecule can be calculated from:

$$60 A = 4 \times 0.855 \left[ \frac{M}{4} \sqrt{2N} d_1 \right]^{2/3} \quad (3)$$

In this equation  $M$  is the weight of the molecule,  $N$  is Avagadro's number and  $d_1$  is the liquid density. By knowing  $V_m$  and the cross sectional area of the adsorbed molecule, the surface area of the sample easily can be calculated.

65 70 75 If an isotherm is started at zero pressure, continued to a relative pressure of one and then desorbed, that is starting at a relative pressure of one and working down toward zero pressure, a hysteresis is often found. The presence of the hysteresis loop is interpreted as showing that the sample has a porous structure. From various analyses of these loops, the size and distribution of the micropores can be obtained.

In brief, the procedure for determining the surface area per unit weight of filament is to determine volumetri-

cally the amount of gas adsorbed on the sample as a function of pressure at the temperature the gas liquifies. The amount of gas required to form a monolayer is calculated by the use of the Brunauer-Emmett-Teller equation. Then, by knowing the cross sectional area of the molecule of the gas, one can calculate the surface area of the filament. The internal surface area of acrylonitrile polymer filaments has been found to be considerable. The ratio of the total surface area to the geometric external area is roughly 500 which indicates a relatively large internal porosity.

The density (apparent) of the filaments either as finished filaments or as they leave the coagulating bath can be determined by mercury displacement. The density data indicate the total porosity of the filaments, including the porosity attributable to the presence of voids and micropores. This void volume data, together with the surface area data and diameter data of the micropores, can be used to calculate the size and frequency of the micropores. At least two techniques are known for determining the density of a filament, these being a pycnometer procedure and a buoyancy procedure. The pycnometer method involves determining the volume of mercury excluded from a calibrated pycnometer by a filament sample. The second procedure comprises determining the loss in weight of a calibrated platinum bob in mercury with and without a filament sample. From the data obtained one may calculate conveniently the density of the sample.

The term "area ratio" refers to the ratio of the measured cross-sectional area of the individual filaments as spun to the cross-sectional area of those filaments as calculated from the denier of the filaments and the known density of the polymer. The filaments prepared in accordance with the present invention possess an unusually low area ratio when the filaments leave the coagulation bath. It is thought that such initially low area ratio is related to the final improved properties of the filaments.

By "acrylonitrile polymer" is meant polyacrylonitrile, copolymers, and terpolymers of acrylonitrile, and blends of polyacrylonitrile and copolymers of acrylonitrile with other polymerizable mono-olefinic materials, as well as blends of polyacrylonitrile and such copolymers with small amounts of other polymeric materials, such as polystyrene. In general, a polymer made from a monomeric mixture of which acrylonitrile is at least 70 percent by weight of the polymerizable content is useful in the practice of the present invention. Besides polyacrylonitrile, useful copolymers are those of 80 or more percent of acrylonitrile and one or more percent of other mono-olefinic monomers. Block and graft copolymers of the same general type are within the purview of the invention. Suitable other monomers include vinyl acetate, and other vinyl esters of monocarboxylic acids, vinylidene chloride, vinyl chloride and other vinyl halides, dimethyl fumarate and other dialkyl esters of fumaric acid, dimethyl maleate and other dialkyl esters of maleic acid, methyl acrylate and other alkyl esters of acrylic acid, styrene and other vinyl-substituted aromatic hydrocarbons, methyl methacrylate and other alkyl esters of methacrylic acid, vinyl-substituted heterocyclic nitrogen ring compounds, such as the vinyl imidazoles, etc., the alkyl-substituted vinyl-pyridines, vinyl chloroacetate, allyl chloroacetate, methylallyl chloroacetate, allyl glycidyl ether, methylallyl glycidyl ether, allyl glycidyl phthalate, and the corresponding esters of other aliphatic and aromatic dicarboxylic acids, glycidyl acrylate, glycidyl methacrylate, and other mono-olefinic monomers copolymerizable with acrylonitrile.

Many of the more readily available monomers for polymerization with acrylonitrile form copolymers which are not reactive with some dyestuffs and may therefore be impossible or difficult to dye by conventional techniques. Accordingly, these non-dyeable fiber-forming

5 copolymers may be blended with polymers or copolymers which are in themselves more dye-receptive by reason of their physical structure or by reason of the presence of functional groups chemically reactive with the dyestuff, whereby the dyestuff is permanently bonded to the polymer in a manner which lends resistance to removal thereof by the usual laundering and dry cleaning procedures. Suitable blending polymers may be polyvinylpyridine, polymers of alkyl-substituted vinylpyridine, polymers of other vinyl-substituted N-heterocyclic compounds, the copolymers of the various vinyl-substituted N-heterocyclic compounds and other copolymerizable monomers, particularly acrylonitrile.

10 Of particular utility are the blends formed of polyacrylonitrile or a copolymer of more than 90 percent acrylonitrile and up to 10 percent vinyl acetate, and a copolymer of vinylpyridine or an alkyl-substituted vinylpyridine and acrylonitrile, the said acrylonitrile being present in substantial proportions to provide heat and solvent resistance, and a substantial proportion of the vinylpyridine or derivatives thereof to render the blend receptive to acid dyestuffs. Of particular utility are the blends of copolymers of 90 to 98 percent acrylonitrile and 10 to 2 percent vinyl acetate and sufficient copolymer of 10 to 70 percent acrylonitrile and 90 to 30 percent vinylpyridine to produce a blended composition with a total of 2 to 10 weight percent vinylpyridine.

15 The polymers just described may be prepared by any conventional polymerization procedure, such as mass polymerization methods, solution polymerization methods, or aqueous emulsion methods. The polymerization is normally catalyzed by known catalysts and is carried out in equipment generally used in the art. However, the preferred practice utilizes suspension polymerization 20 wherein the polymer is prepared in finely divided form for immediate use in the filament forming operations. The preferred suspension polymerization involves batch procedures, wherein monomers are charged with an aqueous medium containing the necessary catalyst and dispersing agents. A more desirable method involves the semi-continuous procedure in which the polymerization reactor containing the aqueous medium is charged with the desired monomers gradually throughout the course 25 of the reaction. Entirely continuous methods involving the gradual addition of monomers and the continuous withdrawal of polymer can also be employed.

30 The polymerization is catalyzed by means of water-soluble salts of peroxy acids, sodium peroxide, hydrogen peroxide, sodium perborate, the sodium salts of other peroxy acids, and other water-soluble compounds containing the peroxy group:

(—O—O—)

35 A wide variation in the quantity of peroxy compound is possible. For example, from 0.1 to 3.0 percent by weight of the polymerizable monomer may be used. The so-called redox catalyst system also may be used. Redox agents are generally compounds in a lower valent state which are readily oxidized to the higher valent state under the conditions of reaction. Through the use 40 of this reduction oxidation system, it is possible to obtain polymerization to a substantial extent at lower temperatures than otherwise would be required. Suitable "redox" agents are sulfur dioxide, the alkali metal and ammonium bisulfites, and sodium formaldehyde sulfoxylate. The catalyst may be charged at the outset of the reaction, or it may be added continuously or in increments throughout the reaction for the purpose of maintaining a more uniform concentration of catalyst in the reaction mass. The latter method is preferred because it tends to make the resultant polymer more uniform in regard to its 45 chemical and physical properties.

50 Although the uniform distribution of the reactants throughout the reaction mass can be achieved by vigor-

ous agitation, it is generally desirable to promote the uniform distribution of reagents by using inert wetting agents, or emulsion stabilizers. Suitable reagents for this purpose are the water-soluble salts of fatty acids, such as sodium oleate and potassium stearate, mixtures of water-soluble fatty acid salts, such as common soaps prepared by the saponification of animal and vegetable oils, the "amino soaps," such as salts of triethanolamine and dodecylmethylamine, salts of rosin acids and mixtures thereof, the water-soluble salts of half esters of sulfonic acids and long chain aliphatic alcohols, sulfonated hydrocarbons, such as alkyl aryl sulfonates, and any other of a wide variety of wetting agents, which are in general organic compounds containing both hydrophobic and hydrophilic radicals. The quantity of emulsifying agent will depend upon the particular agent selected, the ratio of monomer to be used and the conditions of polymerization. In general, however, from 0.1 to 1.0 weight percent based on the weight of the monomers can be employed.

The emulsion polymerizations are preferably conducted in glass or glass-lined vessels provided with means for agitating the contents therein. Generally, rotary stirring devices are the most effective means of insuring the intimate contact of the reagents, but other methods may be successfully employed, for example, by rocking or rotating the reactors. The polymerization equipment generally used is conventional in the art and the adaptation of a particular type of apparatus to the reaction contemplated is within the province of one skilled in the art.

The optimum methods of polymerization for preparing fiber-forming acrylonitrile polymers involve the use of polymerization regulators to prevent the formation of polymer units of excessive molecular weight. Suitable regulators are the alkyl and aryl mercaptans, carbon tetrachloride, chloroform, dithioglycidol and alcohols. The regulators may be used in amounts varying from 0.001 to two percent, based on the weight of the monomer to be polymerized.

The polymers from which the filaments are produced in accordance with the present invention have specific viscosities within the range of 0.10 to 0.40. The specific viscosity value, as employed herein, is represented by the formula:

$$N_{sp} = \frac{\text{Time of flow of polymer solutions in seconds}}{\text{Time of flow of the solvent in seconds}} - 1$$

Viscosity determinations of the polymer solutions and solvent are made by allowing said solutions to flow by gravity at 25° C. through a capillary viscosity tube. In the determinations herein, a polymer solution containing 0.1 gram of the polymer dissolved in 100 ml. of N,N-dimethylformamide was employed. The most effective polymers for the preparation of filaments are those of uniform physical and chemical properties and of relatively high molecular weight.

Referring now to FIGURE 1, a water coagulable solution comprising an acrylonitrile polymer dissolved in N,N-dimethylacetamide, N,N-dimethylformamide, or the like is passed under pressure from a supply tank (not shown) through a conduit 10 and thence through a candle filter 11 wherein undissolved particles and foreign materials in the solution are removed. Ordinarily, gear pumps are used to pump the solution through the filter 11 and to meter same to the spinneret assembly 12. This assembly includes a spinneret 13 and is suitably disposed below the upper surface of the coagulating liquid 14 composed primarily of polyalkylene glycol and contained in an open-top spinning trough or bath 15. The solution may be extruded through a single orifice or a plurality of orifices in the spinneret 13 to form a filament or bundle of filaments 16. The extruded streams of polymer are directed through the liquid 14 for a predetermined and sufficient distance to cause the solution to coagulate as desired. A guide 17 may be employed to define the path taken by the filaments in bath 15. Fresh liquid 14 is supplied to trough 15 through pipe 18 (which may be polyalkylene glycol

or polyalkylene glycol containing a desirable quantity of solvent) and is withdrawn therefrom through pipe 20.

The coagulated filaments are withdrawn by employment of a positively driven roller 21 or other thread advancing means, the peripheral speed of which preferably is synchronized with the extrusion speed so that the filaments during their travel between the spinneret and the rollers may be attenuated, and if desired, attenuated up to the point just short of where filamentary breakage occurs. After passing around roller 21 and an idler roll 22, the filaments are directed into a second spinning trough 23 containing a liquid 24. Fresh liquid is supplied to trough 23 through pipe 25 and is withdrawn through pipe 26. While it is quite possible to employ three or more liquid-containing troughs, only two have been illustrated and described in the interest of simplicity. The filaments before emerging from the liquid in second trough 23 and being directed around a set of positively driven rolls identified by numerals 27 and 28 are passed under guides 30 and 31. The peripheral speed of rollers 27 and 28 can be adjusted so that a predetermined orientation stretch will be imparted to the filaments 16 during their travel in second trough 23.

To roller 27 a washing liquid such as hot water is supplied from a spray or shower head 32, the liquid being collected in a container or tray 33. It will be recognized that the washing operation can be accomplished in more than one stage of the process and by employment of other known washing means. After leaving rollers 27 and 28, the filaments are directed through a liquid in a third trough 34 by being passed under guides 35 and 36. The liquid 37 in this trough is normally water at an elevated temperature. The filaments are withdrawn therefrom by means of a driven roller 38 and associated idle roller 40 operated at a peripheral speed less than that of the peripheral speed of rollers 27 and 28 so that the filaments are permitted to relax substantially completely and thereby to shrink during their travel in trough 34. Fresh water is supplied to trough 34 through an inlet pipe 41 and is withdrawn through an outlet pipe 42. It will be appreciated that other equivalent means may be used to permit the shrinking or relaxing of the filaments. For example, the filaments may be directed around a tapered roller or rollers and progressively led from the end having the larger circumference to the end having the smaller circumference, the rollers being immersed in a liquid or having a liquid applied thereto. Following the relaxing operation the filaments are passed through a finish bath liquid 43 contained in a vessel 44 and composed of a lubricant or like beneficial treating agent. The filaments after being withdrawn from liquid 43 are dried. As illustrated in FIGURE 1 the filaments are continuously directed around a pair of driven drying drums 45 and 46 heated internally with steam or the like. Thereafter, the filaments are subjected to additional operations such as crimping, cutting, and then are collected in the form of staple fiber, continuous filament yarn, or tow.

As can be seen, the acrylonitrile polymer selected is dissolved in N,N-dimethylacetamide, N,N-dimethylformamide or the like to form a spinning solution. This solution is extruded through a spinneret into a coagulating bath composed of polyalkylene glycol.

As pointed out above, the improvement herein is obtained by spinning the polymer solution into a bath composed of polyalkylene glycol. The term "polyalkylene glycol" as used throughout the specification and claims refers to polyethers which may be derived from alkylene oxides or glycols or from other heterocyclic ethers such as dioxolane, and which may be represented by the formula HO(RO)<sub>n</sub>H in which R stands for an alkylene radical such as methylene, ethylene, propylene, etc., and n is an integer of at least four. It will be appreciated that the polyglycol may contain inert substituents; for example, methoxypolyethylene glycol may be employed. Not all of the alkylene radicals present need be the same. Glycols containing a mixture of radicals such as in block

polymers and copolymers are also useful. Similarly, mixtures of polyglycols of differing compositions or molecular weights can be employed. The glycols which are useful in the process of this invention have molecular weights of at least 200 and may have molecular weights as high as 6000. The preferred glycols are the polyethylene glycols which preferably have molecular weights of 600-2000. These glycols as just defined are either viscous liquids or waxy solids at room temperature. However, they become less viscous at higher temperatures and permit spinning at these temperatures. Although wide variations in the spin bath temperatures are permitted, it is preferred that the temperatures be of the order of 50 to 150° C. depending on which glycol is employed.

FIGURE 2 is a drawing prepared from a photomicrograph. This illustrates the normal appearance of acrylonitrile polymer filaments heretofore known at a magnification of 100 times. At this magnification no visible differences between the filaments of the present invention and the known filament are noticeable since the voids or cavities on the surfaces of the filaments are not apparent.

FIGURE 3 is a drawing prepared from a photomicrograph showing a view of part of a filament containing voids or cavities. Enclosed voids of the filament also can be seen by observing a cross section of the filament. Due to the presence of the voids, the light rays impinging thereon are scattered, imparting a dull subdued luster to the filament.

FIGURE 4 is a drawing prepared from a photomicrograph showing a corresponding view of part of a filament substantially free of voids or cavities. Due to the substantial absence of voids, the filament has a lustrous appearance. The novel filaments of the present invention are substantially free of voids and hence have a normally lustrous appearance. However, when desired, delustrants, pigments, and the like can be incorporated in the filaments to produce dull or colored products. The marked differences of the novel filament herein and those heretofore known become apparent when the comparison of the reticulate filamentary structures is made at magnifications obtainable by the use of an electron microscope.

FIGURE 5 is an electron micrograph taken by means of an electron microscopy technique at a magnification of 41,000 times of a longitudinal section of a filament manufactured in accordance with the present invention. The section, as well as other sections whose views appear herein, was prepared using an ultra-microtome fitted with a glass knife. A sample was taken just as the filaments were withdrawn from the coagulating bath. The filament sample was placed in a potentially resinous substance. The substance was polymerized and the polymerized block containing the filament sample was placed in the chuck of a microtome for sectioning. The filament sections were cut and the same were recovered by dissolving the resinous substance in which they were embedded. The thickness of the sections is in the range of 300-600 Å. The filaments in which a sample was taken were manufactured by spinning a solution prepared by dissolving an acrylonitrile polymer in N,N-dimethylacetamide and spinning the solution into the coagulating bath composed essentially of polyethylene glycol having a molecular weight of 1000. The polymer lattice work in the micropores initially existing in the freshly spun filaments can be seen. The frequency and size of the micropores can be noted.

FIGURE 6 is an electron micrograph taken by means of the electron microscopy technique just described. The filament sample viewed is identical to the filament sample in FIGURE 5 except that the filament was stretched 6 times in boiling water. The magnification is 44,000 times. The micropores and the polymer lattice existing in the freshly spun oriented filaments clearly can be seen.

FIGURE 7 is an electron micrograph taken by means of the electron microscopy technique discussed above. The filaments from which the sample was taken were prepared by spinning a solution of acrylonitrile polymer dis-

solved in ethylene carbonate into a coagulating bath composed essentially of polyethylene glycol of a molecular weight of 1000. A comparison of the micropore arrangement and polymer lattice initially existing in the freshly spun filaments shows marked differences in regard to size and frequency of the micropores. The size of the micropores of the filament samples shown in FIGURES 5 and 6 is much smaller as compared with the micropores in the sample shown in FIGURE 7. In addition, the frequency of the micropores of the former sample is greater in number than that of the latter sample.

FIGURE 8 is an electron micrograph of the filament in FIGURE 7 after the filament was given an orientation stretch of 6 times in boiling water. The magnification in this instance is 44,000 times.

FIGURES 9 and 10 illustrate how the outer surfaces of wet spun oriented filaments become frayed by the application thereon of lateral stresses. Filaments exhibiting a higher resistance to abrasion show a less tendency to fray and do not give a premature appearance of wear caused by the expanded polymer lattice. The filaments produced in accordance with the present invention have a higher resistance to abrasion, and accordingly a greater lateral stress is required before the fraying of the polymer lattice becomes manifest.

In FIGURE 11 the large open areas are the voids visible under an optical phase microscope and the small openings are the micropores described above. The difference in the relative sizes of voids and micropores is distinctly evident.

In general, the spinning solution can be prepared by heating and stirring a mixture of a finely divided acrylonitrile polymer of the type described above with a solvent selected from the group consisting of N,N-dimethylacetamide, N,N-dimethylformamide, or the like. The percentage of polymer based on the weight of the solution depends upon the particular polymer or solvent employed as well as the temperature at which the polymer is spun. It is desirable to employ a solution containing a high percentage of polymer for obvious reasons. Ordinarily a solution containing at least 10 percent acrylonitrile is desirable. The spinning solution may be maintained prior to and at extrusion at temperatures from about 20 to 150° C.

Although it is not fully understood how the coagulating bath contributes to the formation of the improved fiber structure, it is believed that the relatively large size of the polyalkylene glycol molecules is such that inflow thereof into the coagulating filaments is minimized whereby denser and more compact filaments are obtained.

Filaments may be given a travel in the coagulating bath, for example, from 2 to 24 inches or more by the employment of a suitably spaced guide and withdrawal rolls as illustrated in FIGURE 1. Between the spinneret and withdrawal rolls, the filaments as indicated above may be subjected to a stretching operation to obtain a desired attenuation thereof, if desired.

A second bath is employed following the coagulating bath wherein the filaments are given a stretch in order to increase the strength as well as otherwise to improve the physical properties of the filaments. This improvement results from an orientation of the polymer molecules along the filament axis. The second bath may consist simply of water, or it may have the same composition as the coagulating bath but at a greater dilution with water. The temperature of the second bath is preferably between 50° and 100° C., the highest feasible temperature being preferred. Draw ratios up to 10 or higher may be employed, the amount of stretch applied depends on the properties desired for the yarn. Preferred draw ratios lie between 1.5 and 8.0.

Following the passage through the coagulating bath and the stretch bath or baths, the filaments are washed substantially free of solvent if desired. This may be accomplished by spraying water on the filaments traveling

around positively driven rolls. The water extracts the solvent from the filaments as they pass gradually from one end of the rollers to the other end. Other equivalent washing means, of course, can be used. Moreover, the washing can be carried out prior to applying the orientation stretch to the filaments as indicated above.

Next the filaments may be permitted to relax, if desired. The resulting filaments which are relaxed in hot or boiling water have higher elongation values as compared to filaments produced in a comparable manner but without being permitted to relax. Surprisingly, the higher elongation values are obtained without a sacrifice of tenacity. Moreover, it appears that an inverse relationship exists between the elongation of the resulting filaments and the temperature at which the filaments are given the orientation stretch. That is to say, for a given orientation stretch, filaments having higher elongation are obtained generally where lower stretch temperatures are employed. As indicated, the step of relaxing is not entirely necessary in accordance with the present invention although in some cases it is to be recommended. Next, the filaments are dried in a conventional manner. This may be done either under tension or under no tension.

Quite unexpectedly the filaments produced by the present invention after leaving the relaxation bath have a substantially reduced porosity and have a smooth mirror-like surface. Hence, the disadvantages associated with drying under tension, such as yellowing of the filaments when subjected to high local temperatures on the drying drums and like apparatus used in a tension drying operation, may be avoided and yet produce filaments having a luster greater than normal wet-spun filaments dried under tension. Moreover, the present process enables one to produce filaments of very fine deniers. Owing to the high jet stretch permitted by the process as pointed out above, filaments having individual filaments as low as 0.25 can be successfully spun.

The following examples in which parts and percentages are given by weight unless otherwise indicated illustrate preferred methods of preparing filaments in accordance with the principles of this invention. The invention is not to be limited by the details set forth in the following examples.

#### EXAMPLE I

A 20 percent solution of a copolymer of 95 percent acrylonitrile and 5 percent vinyl acetate was prepared by intimately mixing the copolymer in powdered form with the solvent, N,N-dimethylacetamide, until a clear liquid resulted. The resulting solution was cooled to a temperature of 50° C., filtered, and extruded through a spinneret submerged in a coagulating bath composed of polyethylene glycol having an average molecular weight of 1000. The filaments so formed were withdrawn from the coagulating bath after a travel therein of 20 inches and thereafter directed through a bath of boiling water where a stretch of 6.0 times was imparted to the filaments. Next, the filaments were dried by passing same around rotating drying cans maintained at a temperature of 125° C. Samples of the filaments were taken at the point where they emerged from the coagulating bath and were centrifuged for 60 seconds to remove excess surface liquids. Analyses for several typical samples are presented below in Table 1. Additional spinnings were conducted using polyethylene glycol having a molecular weight of 600 as the coagulating liquid. This lower molecular weight glycol was employed in the presence of varying amounts of the dimethylacetamide solvent. Also, filaments were produced using an aqueous coagulating bath having the composition of 55 percent N,N-dimethylacetamide and 45 percent water. The results of these spinnings are also given in Table 1.

Table 1

|    | Coagulating Bath Composition                        | Percent Polymer in Sample | Percent Solvent in Sample | Percent Glycol or water in Sample | Percent Original Solvent Extracted |
|----|-----------------------------------------------------|---------------------------|---------------------------|-----------------------------------|------------------------------------|
| 5  |                                                     |                           |                           |                                   |                                    |
|    | Polyethylene glycol (M.W.=1000)-----                | 70                        | 22                        | 8                                 | 90                                 |
|    | Polyethylene glycol (M.W.=600)-----                 | 69                        | 23                        | 8                                 | 89                                 |
| 10 | 95% polyethylene glycol (M.W.=600)+5% Solvent-----  | 61                        | 30                        | 9                                 | 83                                 |
|    | 90% polyethylene glycol (M.W.=600)+10% Solvent----- | 60                        | 25                        | 15                                | 86                                 |
|    | 80% polyethylene glycol (M.W.=600)+20% Solvent----- | 60                        | 23                        | 17                                | 87                                 |
|    | 55% Solvent+45% Water-----                          | 35                        | 35                        | 30                                | 67                                 |

15 The higher polymer content of the filaments spun using the polymeric glycol baths of the present invention is evident; and it can be seen from the above data that the solvent and coagulating liquid contents thereof accordingly are lower. Furthermore, there seems to be very little difference between the solvent content of the filaments spun into a bath of 100% glycol as compared to the solvent content of those filaments spun into baths containing up to 20 percent solvent; and no substantial difference is seen in regard to the solvent content when the molecular weight of the polyethylene is varied. The fact that no significant differences in coagulation rates are indicated when the glycol baths are diluted with 20 percent solvent shows that the solvent level of the coagulating bath can be maintained at a level up to at least 20 percent.

20 Results comparable to those above were obtained by spinning a 20 percent solution of a copolymer blend composed of 85-90 percent of a copolymer of 97 percent acrylonitrile and 3 percent vinyl acetate and a sufficient amount of a copolymer of 50 percent acrylonitrile and 50 percent 2-methyl-5-vinylpyridine to give a total vinylpyridine content by weight of about 6 percent.

25

30

35

40

45

50

55

60

65

70

75

To determine the effect of the molecular weight of the polymeric glycols and of the coagulating bath temperatures on the jet stretch and coagulation of the acrylonitrile polymer filaments, a series of spinnings using various coagulating bath compositions and coagulating bath temperatures were conducted. The copolymer of 95 percent acrylonitrile and 5 percent vinyl acetate was dissolved in N,N-dimethylacetamide to form an 18 percent solution. The solution was extruded through a spinneret having orifices with a diameter of 0.0035 inch.

The effect of increasing bath temperatures and molecular weight of the glycol on the jet stretch can be seen in Table 2 in which the results of using various glycol-containing baths are compared with the results when baths of water and a solvent/water mixture are used.

#### EXAMPLE II

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4875

4880

4885

4890

4895

4900

4905

4910

4915

4920

4925

4930

4935

4940

4945

4950

4955

4960

4965

4970

4975

4980

4985

4990

4995

5000

Table 2

|  | Bath Composition | Bath Temp., °C. | Yarn Appearance | Max. Jet Stretch |
| --- | --- | --- | --- | --- |

<tbl\_r cells="5" ix="1" maxcspan="

There appears to be a general increase in maximum jet stretch as a function of temperature. For low molecular weight baths (water, solvent/water, and ethylene glycol), temperature and not bath composition appears to be the important variable whereas in the polyethylene glycol-containing bath, the effect of bath composition is additive with the thermal effect to give higher stretches with increasing molecular weight at a given temperature.

An opaque appearance of the yarn indicates an internal spongy structure whereas a clear appearance indicates a denser, more homogeneous structure.

Cross-sections of the filament were cut and observed under an optical phase microscope to determine the influence thereon by both the temperature and molecular weight of the polyethylene glycol used in the coagulating bath. For a given bath temperature there is a progressive improvement in the uniformity and surface smoothness of the filaments as the molecular weight of the bath is increased. There is a less pronounced, but still detectable, trend to greater irregularity with increases in temperature for a given glycol bath composition. The typical cross-section of yarn spun into the polyethylene glycol bath is somewhat in the shape of a horseshoe, and the filament is suggestive of a flat ribbon which has been rolled lengthwise until its edges nearly meet.

It was found that the afterstretch is less affected by the bath composition than is the jet stretch. The maximum afterstretch obtainable for the polymer solutions spun in the polymeric glycol bath was in the range of from 7.5 to 10 times and on the average, 8.5 times. The same polymer solution spun in solvent/water mixtures generally gave a maximum afterstretch of less than 7.0 times regardless of bath temperature or solvent-water ratio. This shows that the filamentary structures obtained by the use of the glycol bath are capable of accepting higher stretches than can normally be obtained by employing aqueous coagulating baths.

#### EXAMPLE III

A 20 percent solution of the copolymer of 95 percent acrylonitrile and 5 percent vinyl acetate in N,N-dimethylacetamide was prepared and extruded into coagulating baths composed of polyethylene glycol of 1000 and 4000 molecular weights to determine the effect of the baths on spinning speeds and denier range.

At 95° C. spinning speeds of up to 500 ft./min. were easily obtained. By taking advantage of the wide latitude in jet stretch afforded by the polymeric glycol baths, it was possible to spin deniers from as high as 8 denier per filament down to 0.5 denier per filament and less with the same spinneret. Deniers as low as 0.25 denier per filament were produced from a spinneret having orifices with diameters of 0.002 inch at spinning speeds of 200-250 ft./min. These spinnings caused no unusual spinning problems. With an aqueous bath it was not possible to spin filaments having an individual denier of less than 1.5 under like conditions.

#### EXAMPLE IV

The acrylonitrile polymer solution of Example III was spun into a coagulating bath composed of equal parts of mixed polyethylene glycols having molecular weights of 400 and 1000. A portion of the resulting filaments were passed through a bath containing a yarn lubricant and an anti-static agent; filaments which had not been so treated compared favorably therewith. It was found that even without the application of finish the filaments have a soft, pleasant hand and required only the application of anti-static finish to give satisfactory processability into fabric.

#### EXAMPLE V

A series of spinnings were conducted in which a 20 percent solution of the copolymer of 95 percent acrylonitrile and 5 percent vinyl acetate in N,N-dimethylacetamide was extruded in various coagulating baths as indicated below in Table 3. The values of tenacity and elongation for various fibers spun in the glycol baths, together

with data of comparative controls spun in aqueous baths, are also given in the table.

Table 3

|    | Bath Composition                 | Bath Temp., °C. | Stretch, Times | Filament Denier | Tenacity, g./den. | Elongation, percent |
|----|----------------------------------|-----------------|----------------|-----------------|-------------------|---------------------|
| 5  | 55% solvent+45% water            | 55              | 5.0            | 2.60            | 3.08              | 16                  |
| 10 | Polyethylene glycol (M. W.=200)  | 100             | 5.0            | 2.62            | 2.72              | 23                  |
|    | Polyethylene glycol (M. W.=400)  | 100             | 5.0            | 2.55            | 3.69              | 24                  |
|    | Polyethylene glycol (M. W.=600)  | 100             | 5.0            | 2.43            | 3.76              | 24                  |
| 15 | Polyethylene glycol (M. W.=1000) | 100             | 5.0            | 2.55            | 3.84              | 23                  |
|    | Do                               | 100             | 6.0            | 2.68            | 4.07              | 19                  |
|    | Do                               | 100             | 8.0            | 2.84            | 4.48              | 17                  |
| 20 | 55% solvent+45% water            | 50              | 4.4            | 3.00            | 2.67              | 17                  |
|    | Polyethylene glycol (M. W.=800)  | 95              | 2.0            | 2.82            | 1.98              | 42                  |
|    | Do                               | 95              | 3.0            | 2.88            | 2.80              | 32                  |
|    | Do                               | 95              | 4.0            | 2.90            | 3.08              | 26                  |
|    | Do                               | 95              | 5.0            | 2.94            | 3.97              | 23                  |

As might be expected, the tenacity of the filaments spun into the polymeric glycol baths depends upon the degree of orientation stretch applied to the fiber. Similarly, elongation shows a characteristic inverse relationship to the amount of stretch.

It can be seen from the above data that for a given stretch ratio, filaments spun into the polymeric glycol baths generally show higher values for both elongation and tenacity than the aqueous controls. It is also apparent that the filaments spun into the polymeric glycol baths have a better balance of elongation and tenacity than do the controls.

#### EXAMPLE VI

The acrylonitrile polymer solution of Example III was spun into a coagulating bath composed of polyethylene glycol having an average molecular weight of 4000. The resulting filaments were processed as in Example I with an afterstretch of 7.0 times being imparted to the filaments. The finished filaments had deniers ranging from 4-9 with tenacities of 2.7-3.2 g./den. and elongations of 17-27 percent.

#### EXAMPLE VII

A homopolymer of acrylonitrile was dissolved in N,N-dimethylformamide to form an 18 percent solution of the polymer. The resulting solution was spun into a bath containing polyethylene glycol having an average molecular weight of 1000. Samples were collected with a variety of after-stretches and had physical properties as given in Table 4.

Table 4

| No. | Stretch, Times | Filament, Denier | Tenacity, g./den. | Elongation, percent |
|-----|----------------|------------------|-------------------|---------------------|
| 1   | 3.5            | 3.0              | 2.6               | 32                  |
| 2   | 4.5            | 3.2              | 3.3               | 26                  |
| 3   | 5.5            | 3.2              | 4.3               | 23                  |
| 4   | 6.5            | 3.7              | 4.4               | 21                  |

#### EXAMPLE VIII

The acrylonitrile polymer solution of Example III was extruded into a series of coagulating baths composed of polypropylene glycol of varying molecular weight. The results of these spinnings are summarized in Table 5 below.

Table 5

| No. | Molecular Weight of Bath | Stretch, Times | Filament, Denier | Tenacity, g./den. | Elongation, percent |
|-----|--------------------------|----------------|------------------|-------------------|---------------------|
| 1   | 1025                     | 9.3            | 3.0              | 3.0               | 28                  |
| 2   | 425                      | 7.5            | 2.5              | 4.5               | 19                  |
| 3   | 425                      | 4.5            | 2.5              | 3.8               | 25                  |
| 4   | 425                      | 5.5            | 2.5              | 4.2               | 23                  |
| 5   | 425                      | 6.5            | 2.5              | 4.5               | 20                  |

**17**  
**EXAMPLE IX**

The acrylonitrile polymer solution of Example III was spun into a coagulating bath at 90° C. containing methoxypolyethylene glycol having an average molecular weight of 750. The resulting filaments were aftertreated as in Example I with afterstretches of 4-6 times. The finished filaments had tenacities of 3-4 g./den. and elongations of 20-30 percent.

**EXAMPLE X**

Eighty-eight parts of a copolymer of 95 percent acrylonitrile and 5 percent vinyl acetate were blended with 12 parts of polyvinylpyrrolidone with the resulting blend being dissolved in N,N-dimethylacetamide to form a 20 percent solution. This solution was extruded into a bath composed of polyethylene glycol having an average molecular weight of 1000. The resulting filaments were processed in the manner described in Example I with an afterstretch of 6 times being imparted to the filaments. The finished filaments contained in excess of 10 percent polyvinylpyrrolidone and had improved dye take-up with most dyestuffs. The filaments had a tenacity of 3.9 g./den. and an elongation of 21 percent.

**EXAMPLE XI**

A spinning solution was prepared by dissolving a copolymer of 94 weight percent acrylonitrile and 6 weight percent of vinyl acetate in N,N-dimethylacetamide. Samples of the spinning solution at 30° C. were extruded through a spinneret into a coagulating bath consisting essentially of polyethylene glycol having a molecular weight of 1000 and maintained at 93° C. The filaments were withdrawn from the coagulating bath after the same were directed therethrough for a distance of 24 inches. At this point it was found that the filaments were composed of 42.2 percent acrylonitrile polymer, 9.2 percent N,N-dimethylacetamide, and 48.6 percent of polyethylene glycol. The filaments were then passed through a water wash bath. It was found that the filaments were composed of 47.6 percent acrylonitrile polymer, 2.1 percent N,N-dimethylacetamide, and 50.3 percent water.

For comparison purposes, the same acrylonitrile polymer spinning solution was likewise extruded into an aqueous coagulating bath composed of 55 percent N,N-dimethylacetamide and 45 percent water at 50° C. The filaments removed from the coagulating bath in this instance were composed of 28.7 percent acrylonitrile polymer, 40.0 percent N,N-dimethylacetamide and 31.3 percent water. The filaments were then passed through a water wash bath as above. It was found that the filaments were composed of 26.9 percent acrylonitrile polymer, 0.0+ percent N,N-dimethylacetamide, and 73.1 percent water.

These data indicate that in accordance with the present invention the filaments immediately after coagulation contain a higher percentage of polymer and accordingly are more dense. Moreover, it is manifest that drying of the washed filaments produced by the present invention could readily be accomplished and would require less heat and drying time, as compared with aqueous spun controls. This is due to the lower moisture content in and the initially denser structure of the filaments.

**EXAMPLE XII**

The improvement of the present invention in regard to the abrasion resistance of the filaments when converted into fabric was studied.

A spinning solution was prepared by dissolving in N,N-dimethylacetamide a blend of (A) a copolymer of 97 percent acrylonitrile and 3 percent vinyl acetate with (B) a copolymer of 50 percent acrylonitrile and 50 percent 2-methyl-5-vinylpyridine, said blend containing 6 percent vinylpyridine based on the weight of the blend. The polymer blend had a specific viscosity of 0.25 and the spinning solution contained 18 percent solids. The solu-

**18**

tion was extruded at 50° C. through a spinneret containing 1000 holes, each being 0.003 inch in diameter, into a coagulating bath composed essentially of polyethylene glycol having a molecular weight of 1000. The temperature of the coagulating bath was maintained at 100° C. The bundle of filaments formed was led through the bath for a distance of 36 inches and then was removed therefrom at a rate of 40 feet per minute, the rate of withdrawal being established in relation to the rate of extrusion so that the filaments are subjected to a draw ratio of 1.1 between the spinneret submerged in the coagulating bath and the means used to withdraw the filaments from the coagulating bath. Next the filaments were passed into a second stretch bath maintained at 100° C. and containing essentially water. After they had traveled a distance of 12 inches in the second bath, the filaments were withdrawn at a rate of 140 feet per minute so that a stretch of approximately 3.5 times was imparted to the filaments. The filaments were then passed around a pair of spaced apart rollers 34 to 40 times with a total length of filaments around the rollers at one time being about 120 feet. Water at 50-80° C. was sprayed on the filaments during their travel around said rolls to wash same. Following the washing operation, the filaments were dried by being passed around a heated drum assembly.

In like manner additional filaments were produced under the same conditions as just described except in this instance the filaments were given an orientation stretch of 6.5 times and before drying were directed into a relaxation bath composed of water at 100° C. with the filaments being withdrawn therefrom at a rate such that the filaments are permitted to shrink 10 percent in length.

For additional comparison purposes the polymer spinning solution was spun into an aqueous coagulating bath having the composition of 55 percent N,N-dimethylacetamide (DMA) and 45 percent water. This bath was maintained at 55° C. The filaments were given an orientation stretch of 4.5 times and subjected to an annealing operation as above described.

In each case the resulting filaments were uptwisted 3-5 turns per inch and knitted into a narrow tape 14 ends wide on a tricot knitting machine. The resulting tapes were then tested on a Stoll abrader until failure occurred. The abrasion resistances are tabulated below in Table 6.

*Table 6*

| Bath Comp.                | Percent Relaxation | Cycles to Break |     |
|---------------------------|--------------------|-----------------|-----|
|                           |                    | Wet             | Dry |
| PEG 1000-----             | 0                  | 892             | 620 |
| PEG 1000-----             | 10                 | 1,122           | 766 |
| DMA+H <sub>2</sub> O----- |                    | 316             | 358 |

This study above indicates that one obtains a general improvement in the abrasion resistance when the acrylonitrile polymer filaments are produced in accordance with the present invention. Moreover, the resistance to abrasion of the filaments when wet is somewhat better than that of dry filaments. However, it is to be noted that filaments produced using a conventional aqueous bath had a greater resistance to abrasion when dry than when wet.

**EXAMPLE XIII**

Samples of the spinning solution described above in Example XII were spun into a coagulating bath at 95° C. Baths composed of polyethylene glycols of molecular weights of 1000 and 400 were used. In each instance the filaments were withdrawn from the coagulating bath after the same were directed therethrough for a distance of 24 inches. The rate of withdrawal was established in relation to the rate of extrusion so that the filaments were subjected to a draw ratio of 0.8. The filaments were then washed, collected, frozen, and dried

under vacuum without additional aftertreatment. In Table 7 below fiber surface area data for the filaments so formed are given.

Table 7

| Bath Comp.    | Inner Fiber Surface Area, m. <sup>2</sup> /g. | Fiber Density, gm./cc. | Area Ratio | Pore Diameter, Å. | Pore Frequency <sup>1</sup> |
|---------------|-----------------------------------------------|------------------------|------------|-------------------|-----------------------------|
| PEG 1000----- | 180                                           | 0.81                   | 1.48       | 120               | $3.650 \times 10^{14}$      |
| PEG 400-----  | 141                                           | 0.62                   | 1.89       | 315               | $440 \times 10^{14}$        |

<sup>1</sup> Number of pores per gram of fiber.

For comparison purposes the same spinning solution was spun into an aqueous coagulating bath consisting of approximately 50 percent water and 50 percent N,N-dimethylacetamide. The inner surface area of these filaments produced in accordance with the conventional wet spinning method was 100 m.<sup>2</sup>/gram. Other comparative data were as follows: Fiber density—0.49 gm./cc.; area ratio—2.42; pore diameter—340 Å. and pore frequency— $62 \times 10^{14}$ .

## EXAMPLE XIV

In accordance with a known method the polymer blend described in Example XII was dissolved in ethylene carbonate. The resulting solution contained 19 percent solids. The solution was extruded at 100° C. through a spinneret containing 100 holes, each being 0.0035 inch in diameter, and into a bath containing polyethylene glycol of 1000 molecular weight and maintained at 100° C. The filaments thus formed were washed free of solvent, collected, frozen, and dried under vacuum without additional aftertreatment. The fiber inner surface area was 12.5 m.<sup>2</sup>/gram. Other comparative data were as follows: Fiber density—0.6 gm./cc.; area ratio—1.95; pore diameter—4000 Å. and pore frequency— $2.5 \times 10^{13}$ . Finished filaments gave a very dull appearance.

The present invention makes possible the production of acrylonitrile polymer filaments that have an optimum balance of longitudinal and lateral properties and that are eminently suitable for use in the textile art. The filaments have increased elongation realized without sacrifice of tenacity, higher elongation enabling the filaments to be tougher and to be able to adsorb more energy without breakage. Moreover, the filaments are substantially free from voids and have a highly lustrous appearance. By proper selection of stretch ratios, it is possible according to the present invention to produce a filament equivalent in elongation-tenacity balance to the normally aqueous spun filaments that have been annealed. Consequently by using the high molecular weight glycol bath of the present invention, the annealing step may be eliminated without sacrificing the physical properties of the yarn in regard to balance of elongation and tenacity. It is not necessary according to the present invention to dry the filaments under tension in order to produce a satisfactorily dense fiber structure. Also the present process lends itself readily to employment on a commercial scale without substantial modification of conventional equipment. The surface of filaments spun into a high molecular weight polyalkylene glycol bath of the present invention is relatively smooth and substantially free from the surface pits which characterize filaments spun in aqueous baths. The smooth surface of the filaments results in a very high gloss. The addition of a delustrant, such as titanium dioxide, opaques the filaments but does not mask the surface gloss. Boiling or annealing usually has little effect on the appearance of the filaments.

Drying of the filaments produced for the present invention is readily accomplished and requires little heat. Of importance is the fact that the filaments show less tendency to fibrillate as determined by standard fibrilla-

tion tests and as compared with aqueous spun filaments. Without being annealed, filaments produced in accordance with the present invention have resistances to abrasion comparable to or greater than that of aqueous spun filaments that have been annealed. Numerous other advantages of the present invention will be apparent to those skilled in the art.

Any departure from the description herein that conforms to the present invention is intended to be included within the scope of the claims.

This application is a continuation-in-part of copending application Serial No. 755,372, filed August 18, 1958 (now abandoned).

What is claimed is:

15. A textile-grade, molecularly oriented, normally lustrous filament manufactured from an acrylonitrile polymer and substantially free of porosity, characterized by having an internal fiber surface area in the range of about 150-500 square meters per gram of said filament, said surface area being a measure of engaging surfaces defining collapsed submicroscopic interstitial spaces, the surfaces being spaced apart at a distance of at most about 300 Å., as measured before the orientation of the filament and the collapsing of said spaces, the frequency of said spaces being in the range of about 200-2000×10<sup>14</sup> per gram of said filament.
20. A textile-grade, molecularly oriented, normally lustrous filament manufactured from an acrylonitrile polymer having a specific viscosity of 0.1 to 0.4 and substantially free of porosity, characterized by having an internal fiber surface area in the range of 150-500 square meters per gram of said filament, said surface area being a measure of engaging surfaces defining collapsed submicroscopic interstitial spaces, the surfaces being spaced apart at a distance of at most 300 Å. as measured before the orientation of the filament and the collapsing of said spaces, the frequency of said spaces being in the range 200-2000×10<sup>14</sup> per gram of said filament, the average number of said spaces per millimeter of length of said filament taken along a longitudinal plane being at least 40,000.
25. A continuous filament yarn composed of a plurality of filaments described in claim 2.
30. A spun yarn composed of a plurality of staple fibers made from filaments described in claim 2.
35. A textile-grade, molecularly oriented, normally lustrous filament manufactured from a copolymer of at least 80 percent by weight acrylonitrile and up to 20 percent of another mono-olefinic monomer and substantially free of porosity, characterized by having an internal fiber surface area of about 150-500 square meters per gram of said filament, said surface area being a measure of engaging surfaces defining collapsed submicroscopic interstitial spaces, the surfaces being spaced apart at a distance of at most 300 Å. as measured before the orientation of the filament and the collapsing of said spaces, the frequency of said spaces being about 200-2000×10<sup>14</sup> per gram of said filament, the average number of said spaces per millimeter of length of said filament taken along a longitudinal plane being at least 40,000.
40. The filament described in claim 5 wherein the mono-olefinic monomer is vinyl acetate.
45. A continuous filament yarn composed of a plurality of filaments described in claim 6.
50. A textile-grade, molecularly oriented, normally lustrous filament manufactured from a polymer blend of a copolymer of 80 to 99 percent acrylonitrile and 20 to 1 percent of another mono-olefinic monomer and a copolymer of 10 to 70 percent acrylonitrile and 90 to 30 percent of a vinyl-substituted tertiary heterocyclic amine, said blend having an overall vinyl-substituted tertiary heterocyclic amine content of 2 to 10 percent based on the weight of the blend and substantially free of porosity, characterized by having an internal fiber surface area of 150-500 square meters per gram of said filament, said surface area being a measure of engaging surfaces defining

collapsed submicroscopic interstitial spaces, the surfaces being spaced apart at a distance of at most 300 Å. as measured before the orientation of the filament and the collapsing of said spaces, the frequency of said spaces being  $200-2000 \times 10^{14}$  per gram of said filament, the average number of said spaces per millimeter of length of said filament taken along a longitudinal plane being at least 40,000.

9. A textile-grade, molecularly oriented, normally lustrous filament manufactured from a copolymer of at least 80 percent by weight acrylonitrile and up to 20 percent of another mono-olefinic monomer and substantially free of porosity, characterized by having an internal fiber surface area of 150-500 square meters per gram of said filament, said surface area being a measure of engaging surfaces defining collapsed submicroscopic interstitial spaces, the surfaces being spaced apart at a distance of at most 300 Å. as measured before the orientation of the filament and the collapsing of said spaces, the frequency of said spaces being  $200-2000 \times 10^{14}$  per gram of said filament, the average number of said spaces per millimeter of length of said filament taken along a longitudinal plane being at least 40,000 and further characterized by displaying a higher resistance to abrasion when wet than dry.

10. A textile-grade, molecularly oriented, normally lustrous filament manufactured from a polymer blend of a copolymer of 80 to 99 percent acrylonitrile and 20 to 1 percent of another mono-olefinic monomer and a copolymer of 10 to 70 percent acrylonitrile and 90 to 30 percent of a vinyl-substituted tertiary heterocyclic amine, said blend having an overall vinyl-substituted tertiary heterocyclic amine content of from 2 to 10 percent based on the weight of the blend and substantially free of porosity, characterized by having an internal fiber surface area of 150-500 square meters per gram of said filament, said surface area being a measure of engaging surfaces defining collapsed submicroscopic interstitial spaces, the surfaces being spaced apart at a distance of at most 300 Å. as measured before the orientation of the filament and the collapsing of said spaces, the frequency of said spaces being  $200-2000 \times 10^{14}$  per gram of said filament, the average number of said spaces per millimeter of length of said filament taken along a longitudinal plane being at least 40,000 and further characterized by displaying a higher resistance to abrasion when wet than dry.

11. A textile-grade, molecularly oriented, normally lustrous filament manufactured from a copolymer of at least 80 percent by weight acrylonitrile and up to 20 percent of another mono-olefinic monomer and substantially free of porosity, characterized by having an internal fiber surface area of 150-500 square meters per gram of said filament,

said surface area being a measure of engaging surfaces defining collapsed submicroscopic interstitial spaces, the surfaces being spaced apart at a distance of at most 300 Å. as measured before the orientation of the filament and the collapsing of said spaces, the frequency of said spaces being  $200-2000 \times 10^{14}$  per gram of said filament, the average number of said spaces per millimeter of length of said filament taken along a longitudinal plane being at least 40,000 and further characterized by displaying a higher resistance to abrasion when wet than dry and by requiring a tension of at least one gram per denier to be elongated 5 percent in water at 100° F.

12. A textile-grade, molecularly oriented, normally lustrous filament manufactured from a polymer blend of a copolymer of 80 to 99 percent acrylonitrile and 20 to 1 percent of another mono-olefinic monomer and a copolymer of 10 to 70 percent acrylonitrile and 90 to 30 percent of a vinyl-substituted tertiary heterocyclic amine, said blend having an overall vinyl-substituted tertiary heterocyclic amine content of 2 to 10 percent based on the weight of the blend and substantially free of porosity, characterized by having an internal fiber surface area of 150-500 square meters per gram of said filaments, said surface area being a measure of engaging surfaces defining collapsed submicroscopic interstitial spaces, the surfaces being spaced apart at a distance of 10 to 300 Å. as measured before the orientation of the filament and the collapsing of said spaces, the frequency of said spaces being  $200-2000 \times 10^{14}$  per gram of said filament, the average number of said spaces per millimeter of length of said filament taken along a longitudinal plane being at least 40,000 and further characterized by displaying higher resistance to abrasion when wet than dry and by requiring a tension of at least one gram per denier to be elongated 5 percent in water at 100° F.

13. A continuous filament yarn composed of a plurality of filaments described in claim 11.

14. A spun yarn composed of a plurality of staple fibers made from filaments described in claim 12.

#### References Cited in the file of this patent

##### UNITED STATES PATENTS

|           |                 |                |
|-----------|-----------------|----------------|
| 2,268,160 | Miles           | Dec. 30, 1941  |
| 2,764,468 | Hare            | Sept. 25, 1956 |
| 2,788,563 | Stuchlik et al. | Apr. 16, 1957  |
| 2,821,458 | Evans           | Jan. 28, 1958  |
| 2,826,566 | Bruson          | Mar. 11, 1958  |
| 2,880,056 | Carr et al.     | Mar. 31, 1959  |
| 2,907,096 | Halbig          | Oct. 6, 1959   |
| 2,948,048 | Jankens         | Aug. 9, 1960   |